

## UNITED STATES PATENT OFFICE.

BENNETT GROTTA, OF TAMAQUA, PENNSYLVANIA, ASSIGNOR TO ATLAS POWDER COMPANY, OF WILMINGTON, DELAWARE, A CORPORATION OF DELAWARE.

## COMPOSITION FOR DETONATORS.

No Drawings.

Application filed November 25, 1921. Serial No. 517,661.

To all whom it may concern:

Be it known that I, BENNETT GROTTA, a citizen of the United States, residing at Tamaqua, in the county of Schuylkill and 5 State of Pennsylvania, have invented certain new and useful Improvements in Compositions for Detonators, of which the following is a specification.

My invention relates to improvements to 10 that class of detonators which contain a heavy metal azide as a whole or as a part of the charge.

For many years efforts have been made to effect improvements in detonators, by substituting some ingredient, either wholly or partially, for fulminate of mercury, the latter compound having been the chief initiating explosive of commercial importance since its discovery.

20 Fulminate of mercury is superior to all known commercially possible detonating explosives in one respect, in that detonation is assured, either by the spit of a fuse or other means of ignition, or by moderate percussion. On the other hand, fulminate of 25 mercury exhibits several undesirable properties: (1) It is easily affected by moisture, a fraction of one percent of water content being sufficient to destroy its detonating value. (2) Its true detonating

30 value is greatly diminished when compressed to high densities as is often times inevitable in the modern methods of manufacturing detonators. (3) It has a relatively low "brisance" or detonating value which renders necessary the use of an "inner capsule" or re-inforced shell when it is desired to use fulminate of mercury as a priming charge in the T. N. T., tetryl, or 35 other nitrocompound types of detonators; a fact which is well known to all who are conversant in this branch of the explosives industry. (4) Due to the corrosive action of fulminate of mercury the number of 40 metals or alloys which are suitable for detonator casings is greatly restricted.

In contrast with fulminate of mercury there is another group of initiating explosives, namely, the heavy metal azides, which 45 have several properties that are directly the reverse of those of fulminate of mercury. The azides are salts of hydrazoic acid which were discovered and, according to literature, were proposed as substitutes for

fulminate of mercury before the year 1900. 55 These compounds are scarcely affected by moisture or over-pressing and they possess much greater brisance or detonating value than fulminate of mercury.

On the other hand, the azides, especially 60 lead azide which has been recognized as the only azide of commercial importance, has the disadvantage of not being easily ignited. As was stated above, fulminate of mercury is ignited with certainty by the spit of a 65 fuse or other means commonly employed in practice. Lead azide, however, exhibits greater stability to heat and requires about twice as high a temperature to initiate detonation as does fulminate of mercury. The 70 flash-point, that is, the lowest temperature which is just sufficient to effect detonation of lead azide is about 330° C., while the flash-point of fulminate of mercury is only about 160° C. Consequently, the applica- 75 tion of lead azide as a primary initiating explosive is limited, for ignition is not assured by the methods commonly employed in practice. Thus it is evident that with respect to those properties in which ful- 80 nimate of mercury is deficient, the azides excel and also that the chief point in favor of fulminate, its ease of ignition, is lacking in the azides.

Because of the above described conditions, it is highly desirable to provide a detonator charge which will embody the merits of the azides, and in which the deficiencies of the azides, (i. e., the high temperature required to initiate detonation) 85 will be supplied by fulminate of mercury. Presumably, such a detonator charge would result from a mixture of fulminate with an azide. A review of the history of detonating explosives, however, reveals the fact 90 that such a proposition has been suggested in 1911 (U. S. Patent No. 1,128,394.)

The reason that, after a period of ten years or more, the commercial and technical practicability of such a proposition has not 100 been demonstrated is as follows:

Different metals or alloys which are suitable for detonator casings or shells in most cases react oppositely with fulminate of mercury and lead azide so that as a rule a 105 shell material which is satisfactory for one compound is highly unsatisfactory for the other. For instance, fulminate of mercury

can be used in copper shells, but, due to electrolytic or chemical action, it effects a rapid corrosion of zinc or aluminum shells. Similarly, lead azide may be used in aluminum shells, but cannot be used in copper shells because, in contact with copper, lead azide forms a dangerously sensitive copper azide. Thus it is evident that a mixture of these two compounds cannot be used in shells 10 made of certain non-sparking metals, such as copper and aluminum, because the metal which would be suitable for the one compound would be attacked by the other.

The above explanation is fully confirmed 15 by experiments and by the fact that there is now being marketed a tetryl detonator, primed with lead azide, which, in turn, is covered with a third charge of an easily-ignitable substance, other than fulminate of 20 mercury, all of which is contained in an aluminum shell. Therefore, it would appear that all hopes of utilizing a mere mixture of fulminate and an azide had been abandoned.

25 Through experimentation, I have discovered that a certain metal salt of hydrazoic acid, other than lead azide, and which has heretofore been considered impractical for technical application, may be mixed with 30 fulminate of mercury, with or without the addition of potassium chlorate, producing the desired results. The azide which I have found suitable for this purpose is the mercurous salt of hydrazoic acid.

35 Although the mercury salts of hydrazoic acid have been considered too dangerous to have practical importance I have found that the mercurous compound, in contradistinction to the mercuric azide, can be made by 40 methods which will produce a comparatively safe product. Mercurous azide is admirably suited for admixture with mercury fulminate because, in the first place, both compounds being salts of the same metal

45 may be mixed without danger of chemical action, and in the second place, there is no appreciable action between such a mixture and shells which would be suitable for fulminate detonators. Throughout exten-

50 sive experimentation I have found that the mercurous compound, in contradistinction to lead azide, does not form the super sensitive copper azide. Even in a moist atmosphere of carbon dioxide, copper is not 55 appreciably attacked by mercurous azide, while, under similar conditions, lead azide very rapidly gives rise to the dangerous copper compound. The secret of this chemical inactivity of mercurous azide has two 60 possible explanations, either of which may be dependent on the other.

1. The comparative positions of the metals involved, in the electro-motive series.

2. The comparative solubilities of mercurous azide and lead azide in water.

It is a well known fact that the mutual reactivity of different salts and metals is largely dependent on the positions of the metals involved in the electromotive series, with respect to hydrogen. In general the wider the gap between two metals, the more rapid will be the reaction. The following table of specific electrode potentials indicates a positive potential value for both aluminum and lead and negative values for copper and mercury. This is in accord with the fact that mixtures of lead azide and fulminate of mercury cannot be used in either copper or aluminum shells.

| Metals.  | Electrode potential. | 80 |
|----------|----------------------|----|
| Aluminum | * +1.040             |    |
| Lead     | ** +0.12             |    |
| Copper   | -0.51                |    |
| Mercury  | -0.80                | 85 |

\* Neumann, Zeitschrift fur Physik, chemie 14, 229.

\*\* Noyes & Sherill, Principles of Chemistry, p. 164.

It is also a well known fact that no metal can displace another metal from a salt unless water or other solvent be present. 90 Therefore the relative solubilities of two difficultly soluble salts should furnish an index of their comparative reactivity with respect to a metal. I have found by actual experiments that mercurous azide is soluble 95 in water at ordinary temperature to the extent of 0.03 grams per liter, while lead azide, under the same conditions, is soluble to the extent of 0.38 grams per liter. A small amount of water is almost unavoidably 100 present in a detonator charge, remaining from a previously wet condition of the ingredients, or from being supplied from the moisture in the air, or both. The fact that lead azide is more than twelve times as 105 soluble as mercurous azide is also in accord with the much greater tendency of lead azide to have its metal displaced by certain other metals, such as copper.

The action of carbonic acid must also be 110 considered. Carbon dioxide is present in the atmosphere. In combination with water it forms carbonic acid, which may act upon the azide with the liberation of the gaseous hydrazoic acid, which in turn may act upon the copper of the shell, with the formation of the dangerous copper azide. The above figures show that mercurous azide is almost insoluble. Thorough and exhaustive tests in an atmosphere of carbon dioxide and 115 moisture have shown that copper or gilding metal shells with mercurous azide do not form this dangerous compound in a detectable amount, even over a long period of time. Lead azide, on the other hand, under the 120 same comparative conditions quickly forms a deposit of this super-sensitive compound.

Further, under the influence of moisture and carbon dioxide, lead azide may be converted to a non-explosive mass, while, under 130

the same conditions, mercurous azide is not noticeably affected. It is well known that ordinary air contains moisture and carbon dioxide and that mine air often contains even greater amounts.

In addition to being wholly practical from a standpoint of stability, I have found that from a standpoint of detonating efficiency, the admixtures of small quantities of mercurous azide with fulminate of mercury, produces most gratifying results. By extensive experimentation I have also found that the advantageous effects of such mixtures hold equally true when the mixtures include suitable proportions of potassium chlorate. The addition of potassium chlorate to the primary detonating composition in detonators is a well known and common procedure. These advantages may be summarized as follows.

1. The brisance or detonating value is greatly increased. The inner capsule, which is essential in a mercury fulminate-tetryl detonator, may be dispensed with, and a smaller priming charge used effectively.

2. Such mixtures are practically unaffected by moisture, whereas mercury fulminate or mercury fulminate-potassium chlorate alone are easily and quickly made ineffective by moisture.

3. Detonators charged with such mixtures are unimpaired by pressures at which fulminate of mercury or fulminate of mercury-potassium chlorate mixtures become "dead pressed."

4. Such mixtures retain the same property of ease of ignition as does straight mercury fulminate, the flash point of various mixtures being practically identical with that of fulminate of mercury. Having described in detail the principles involved in my invention, I will now give specific examples which illustrate its application.

(1) A charge of 1,000 grams of 90-10 fulminate-mercurous azide mixture is charged and pressed into a copper or gilding metal shell.

(2) A charge of 1,000 gram of 80-20 mercury fulminate-mercurous azide mixture is charged and pressed into a copper or gilding metal shell.

(3) A main charge of 0.50 gram of T.N.T., tetryl, or other nitro aromatic explosive is charged and pressed into a copper or gilding metal shell. This main charge is primed with a charge of 0.30 gram of an 80-20 fulminate of mercury-mercurous azide

mixture. An "inner capsule" is not required.

(4) A main charge of 0.50 gram of tetryl is charged and pressed into a copper or gilding metal shell. This main charge is primed with 0.30 gram of a mixture which consists of 80 parts fulminate of mercury, 10 parts of mercurous azide, and 10 parts of potassium chlorate.

While I have given specific examples of the use of mixtures of fulminate of mercury and mercurous azide in detonator compositions, it is to be understood that my invention is not limited to any particular detonator composition or to any specific methods of use in blasting caps or other means of initiating detonation, but that I desire to claim in the broadest manner the use of mixtures of fulminate of mercury and mercurous azide, with or without the addition of other ingredients.

While I have mentioned T. N. T. or tetryl as a main detonator charge combined with a priming charge of fulminate and mercurous azide other compositions may be used in lieu of the T. N. T., such, for example, as hexanitrodiphenylamine, with or without potassium chlorate or other oxidizing agent.

Having described my invention, what I claim is:

1. A detonator charge containing fulminate of mercury and mercurous azide. 90

2. A detonator charge containing fulminate of mercury, mercurous azide and an oxidizing agent.

3. A detonator charge comprising a priming charge of a mixture of mercurous azide and fulminate of mercury, in conjunction with a suitable secondary charge. 95

4. A detonator charge comprising a priming charge of a mixture of mercurous azide, fulminate of mercury and potassium chloride, and a suitable secondary charge. 100

5. A detonator charge containing fulminate of mercury, mercurous azide, and potassium chlorate.

6. A detonator charge containing fulminate of mercury, mercurous azide, potassium chlorate, and T. N. T.

In testimony whereof I affix my signature in the presence of two witnesses.

BENNETT GROTTA.

Witnesses:

VERDA GROTTA,  
RUSSELL M. COOK.